

Oct. 29, 1940.

F. J. TONE

2,219,853

PRODUCTION OF ABRASIVE MATERIAL

Filed Dec. 31, 1935

Fig. 1.



Fig. 2.



Fig. 3.



Fig. 4.



INVENTOR.  
FRANK J. TONE

BY

*R. C. Bunner*  
ATTORNEY.

## UNITED STATES PATENT OFFICE

2,219,853

## PRODUCTION OF ABRASIVE MATERIAL

Frank J. Tone, Niagara Falls, N. Y., assignor, by  
mesne assignments, to The Carborundum Com-  
pany, Niagara Falls, N. Y., a corporation of  
Delaware

Application December 31, 1935, Serial No. 56,843

2 Claims. (CL 51—278)

This invention relates to the production of coated flexible abrasive articles wherein there is employed a backing material containing a plurality of layers.

5 Coated abrasives of the character with which this invention is concerned have been employed in the manufacture of abrasive discs which are commonly used on portable grinders for various purposes such as smoothing down metallic welds.  
10 Due to the manner in which such discs are used, it is necessary that the backing thereof shall have a certain degree of rigidity or stiffness and yet which shall be capable of repeated flexing, since the discs are pressed against the work.  
15 to a degree which causes contact with the work on an area only about 1" wide at the periphery of the discs. Since the discs are operated at speeds upwards of 2000 R. P. M., they must be capable of alternately bending and straightening out at the same rate and for considerable periods of time. It will therefore be seen that discs which are to be subjected to such treatment must possess the ability to be repeatedly flexed while they are under considerable side pressure resulting  
20 from the contact of the disc with the work.  
25

Heretofore it has been customary to make such discs by combining a heavy grade of cloth with a particular type of cellulosic material commonly referred to as vulcanized fiber or hydrolyzed cellulose. This combining is accomplished by coating the surfaces which are to be joined together with glue, uniting the two surfaces, and then subjecting the article to a careful treatment for drying out the glue. After the backing has been thus prepared, it is coated with abrasive grains and glue in the manner shown in the art of making abrasive coated paper or cloth.

30 Vulcanized fiber and the method used to combine it with the cloth are both expensive and the discs are therefore correspondingly costly. Furthermore, since glue cannot be heated much above 150° F. without destroying its strength, and since a combination backing united with glue puffs up and becomes entirely useless if heated much above this point, such backings are entirely unsuited for abrasive products wherein there is employed a binder for the abrasive grains which requires heat treatment above 150° F.

35 It is accordingly an object of the present invention to provide a backing material which shall not be open to the objections enumerated above. It is also an object of the invention to provide a coated abrasive article which shall have the properties required of discs as detailed above and  
40 which shall be relatively inexpensive. Another

object of the invention is to provide an improved method for making coated abrasive articles.

In carrying out my invention I may employ any of a number of kinds of backing material which are to be united into a composite backing. For 5 example, I may use a combination of a heavy grade of cloth with certain special grades of paper or I may use a lighter grade of cloth and I may even use vulcanized fiber in certain special cases where discs are subjected to unusually severe treatment. I may also use combinations of various cloths or combinations of various papers. The backing material may be other materials than cellulosic such as paper or cloth. For example, sheets of dense homogeneous organic material such as resins and cellulosic derivatives may be used. Sheet metals such as sheet steel may also be used.

55 Regardless of the types of backing materials which I may combine, I employ as a binder for 20 uniting these backing layers into a composite article a material which is capable of being softened when heated to a temperature which will not injure the backing material used. There are a number of such materials which are suitable, 25 for example, certain copolymers of vinyl chloride and vinyl acetate which are marketed under various trade names such as "Vinyloid" or "Gelva"; similar vinyl polymers which have been subsequently reacted with acetaldehyde or formaldehyde; cellulose ester lacquers which comprise a cellulose ester such as cellulose nitrate or acetate dissolved in a suitable solvent, usually modified with a plasticizing agent and containing a resin to promote adhesion; polymerized styrol 30 or vinyl benzene, sometimes called meta styrene, which may be modified by plasticizing or flexibilizing agents if desired. In general there may be used materials of this kind which have the property of softening and becoming flexible 35 when heated and hardening again when cooled to normal temperatures.

40 In making up my new backing material I may use any convenient method for applying the binder material to the backing, as for example, by 45 spreading on a solution of the binder by means of a roll in the manner commonly employed in making abrasive paper, or by spraying. Or I may use the binder in the form of a powder in which case I preferably moisten the surface of the back- 50 ing material to which the powder is to be applied, as for example, by wetting the backing with water or with a solvent for the backing binder and then dusting on the powdered binder in a conventional manner.

After applying the binder to a surface of either one or both of the layers which are to be united to form the backing, I then unite these layers by pressing them together in any convenient manner, as for example, by passing them between calender rolls. The calender rolls may be heated if the binder is not sufficiently adhesive at ordinary temperatures. Since it is necessary, in making discs of this type, that the backing shall be relatively stiff and inflexible, I choose such 10 backing materials and employ such a quantity of binder that the completed backing shall be of the desired degree of stiffness.

These binders are, at room temperature, so 15 non-resilient that the backing is so stiff as to be practically impossible to coat satisfactorily in the abrasive paper-coating machine which is customarily used to coat fabrics such as paper or cloth. The use of a thermoplastic resin therefore has the important advantage that the 20 backing made thereof can be made amenable to the operation of the making machine by maintaining it at an elevated temperature whereby the resin is rendered plastic and the backing flexible so 25 that it can be put through the coating machine without cracking and in a manner to apply a satisfactory abrasive coating.

If the combining operation does not warm the resin sufficiently to render the resulting backing sufficiently flexible or if it is desired to have time 30 elapse between the manufacture of the backing and the coating operation the backing may be flexibilized before use by warming. This warming may be done to a roll which has been wound up from a backing as made in the combining 35 machine, or the backing may be fed from the combining machine through a heated chamber. However the combining step may be such that it is warmed to the required degree in the combining 40 machine.

Having rendered the backing material flexible, either in the combining operation or separately, I then coat it with abrasive grains and a binder for the grains, in any convenient manner as carried out in the usual abrasive paper-coating 45 machine. As is well known in the art, this method comprises passing the backing between the so-called pressure roll and the adhesive roll which is partially immersed in a vat of adhesive, and 50 then sprinkling abrasive grains onto the adhesive coated side of the backing. A subsequent sizing coat of adhesive may be, and usually is, applied over the abrasive grains to fix them more firmly on the backing.

Other suitable methods of coating may also 55 be used, e. g., spreading a mixture of adhesive and grain on the backing, or spraying the making or sizing coats, or both, onto the backing.

The invention will be further described with 60 reference to the accompanying drawing, wherein:

Figure 1 is a side view of an abrasive coated article made in accordance with the invention;

Figure 2 is a diagrammatic side section of apparatus suitable for use in carrying out the invention;

Figure 3 is a diagrammatic side section of apparatus suitable for use in carrying out the invention; and

Figure 4 is a diagrammatic side section of apparatus suitable for carrying out the invention.

Referring to the drawing, the coated abrasive article illustrated in Figure 1 comprises a backing material consisting of a layer 1 of cloth cemented to a layer 2 of cellulosic material by a layer 3 of 75 thermoplastic cement. The combination back-

ing is coated with abrasive grains 4 which are attached to the cloth side of the backing by a binder 5.

In Figure 2 I have illustrated apparatus adapted for combining two layers of backing material. In this drawing the roll of cloth 6, mounted on a spindle 7, is fed between adhesive roll 8 and pressure roll 9. The adhesive roll 8 is partially submerged in a body of adhesive 14 contained in a vat 15. The coated web than passes over a heating element 10 and meets a web 11 of cellulosic material supplied from a roll 12 which is mounted on a spindle 13. The heating element 10 is provided with suitable terminals 19 and 20 which are connected to a source of electric potential. 15 The web of cellulosic material and the adhesive coated cloth are passed between rolls 16 and 17, whereby the two layers of backing material are pressed together, and then wound up into a roll 18. 20

Passage of the adhesive coated web over the heating element causes evaporation of the solvent from the adhesive 14 and warms the adhesive to an extent sufficient to cause it to become firmly attached to the cellulosic material 11 and 25 also keeps the adhesive sufficiently flexible so that the subsequently formed backing material can be wound into a suitable roll 18.

In Figure 3 I have illustrated a method of coating my combination backing with abrasive grains. 30

Referring to this drawing, the backing material, wound into a roll 18, suitably warmed to flexibilize the backing adhesive 14, is fed between a grain binder roll 21 and a pressure roll 22. The roll 21 is partially submerged in an adhesive 23 35 which is kept in a suitable vat 24. Rotation of the roll 21 causes a coating of adhesive to be applied to the under side of the backing material and the moving backing material is then passed around an idler roll 25 and under a grain feed 40 hopper 26. The hopper 26 is provided with a gate 27 for adjusting the flow of abrasive grain to a grain feed roll 28. The abrasive grain fed from the hopper by the grain feed apparatus falls onto the abrasive coated web and the coated web 45 then passes around idler rolls 29, 30, 31, 32 and 33, to a suitable festooning apparatus of a type commonly used in the manufacture of abrasive coated webs. The festooning apparatus permits the storage of a relatively large quantity of coated 50 material for a time sufficient to harden the adhesive to a point where the abrasive coated article can be wound up into a roll 34.

The abrasive coated web may be later given 55 an additional coating of adhesive to attach the abrasive grains more firmly to the backing in apparatus similar to that described in Figure 3 or by other suitable means, as for example, by spraying on a sizing coating with the conventional spray gun.

The production of a composite backing material and the steps of coating it with abrasive and adhesive may be carried out continuously in a suitable apparatus. Referring to Figure 4, I have illustrated one apparatus which may be used 65 for making and coating the composite backing in successive steps. A web of cloth 6 which is rolled on spindle 1 is unrolled and coated with thermoplastic adhesive by passing it over fountain roll 8. The coated web is then joined to a web 12 of cellulosic material such as paper which is rolled on a spindle 13. This material is unrolled and passed, together with the coated cloth, between rolls 17 and 16 which press the webs together to cause them to adhere and form a com- 70 75 75

posite sheet. The composite sheet then passes over fountain roll 24 which puts thereon a coating of the adhesive to be used for fixing abrasive grain on the sheet. Abrasive grain is supplied from hopper 26 and the sheet or web is pulled by suction roll 37 to the festooning apparatus wherein it is looped over rods 36 which are carried continuously through the drying or curing chamber. In these festoons the composite backing may be kept warm to keep the cement between the constituent sheets plastic whereby the backing remains flexible so that it can be properly rolled up at the end of the drying or curing stage. If this is incompatible with the proper curing of the adhesive for the abrasive material the backing may be permitted to become cool and stiff during the curing operation, after which it is warmed to flexibilize it before removal from the festoons or before winding up on suitable rolls.

After the backing has been suitably coated with abrasive grains the abrasive coated backing is subjected to a suitable after-treatment to set up the adhesive. Where the adhesive requires a treatment for the evaporation of a solvent this treatment consists in maintaining the article in a chamber suitably controlled as to temperature so as to dry out the binder to the desired degree, and where a heat hardenable binder for the grains is used, the article is heat treated to cure the binder. This after-treatment may be applied to the material while suspended as festoons, or it may be wound in rolls and subjected to the treatment in that form, or the web of coated abrasive may be cut up into suitable shapes such as discs, and the individual discs suitably treated according to a procedure which is commonly employed in the manufacture of abrasive discs.

The materials which may be used for my invention include the papers, cloths and adhesives ordinarily used in making abrasive coated paper and cloth. However the following examples illustrate the invention as applied to the manufacture of sheet material for the manufacture of abrasive discs.

*Example I*

A grade of cloth which is commonly employed in the manufacture of abrasive cloth and known as two eighty five drill (2.85 yds., 30 in. wide, weighs one pound) is moistened with water and a coating of pulverized resin made by hydrolyzing a copolymer of vinyl chloride with vinyl acetate and acetaldehyde is dusted on the moistened cloth. The cloth is then fed through heated calender rolls along with a web of a heavy grade of paper stock where the resin is softened by the heat and caused to stick to both the cloth and the paper and unite them into a composite article. The composite backing is then fed directly into an abrasive paper-making machine and the cloth side of the backing coated with a normally liquid phenolic condensation product resin and abrasive grains, following which a sizing coating of liquid resin is sprayed onto the coating.

The thus formed article is heat treated at 180° F. for two hours to partially set up the liquid resin grain binder, following which discs are cut from the web and subsequently cured at 250° F. for six hours to complete the hardening of the grain binder.

*Example II*

A grade of cloth of the character described in Example I is coated with a cellulose ester lacquer in the form of a solution of cellulose ester

and resin in mixed solvents. The cloth is then warmed to remove most of the solvent, fed through calender rolls along with the web of paper as described in Example I, and then wound up into a roll. This composite backing is rather stiff and inflexible at ordinary room temperatures.

*Example III*

Cloth of the character described in Example I is coated with a solution of a thermoplastic alkyd resin, resulting from the reaction of glycol and a dibasic acid. The cloth is warmed to remove most of the solvent and passed between heated calender rolls with paper to form a composite back.

*Example IV*

Cloth of a suitable character is coated with a solution of a thermoplastic resin resulting from the polymerization of methyl methacrylate. The cloth is warmed to evaporate solvent and make the coating sticky and is then passed between heated rolls with paper to press the cloth and paper together to form a composite sheet.

If the backing thus formed is not used immediately it may be permitted to cool and warmed when wanted for use by putting it in an oven at 200° F. When soft enough it is coated with abrasive grains and a binder in the manner described in Example I, the binder being an air-drying varnish comprising an oil-modified phenolic resin taken up in a drying oil and thinned with solvent.

The abrasive coated material is then further treated to set up the grain binder, and cut up into discs, after which further treatment may be given to complete the hardening of the binder.

As indicated above, by selecting a suitable backing binder and applying a layer of binder of suitable thickness, it is possible to prepare a backing having the required properties of stiffness and flexibility so that the coated backing will be suitable for use in discs of the character described. It is thus possible to vary selectively the flexibility in a series of related articles of this nature whereby a backing material having the flexibility desired for the work may be selectively produced. This may be done by selectively modifying the properties of the backing binder by the addition of suitable agents such as plasticizers like tricresyl phosphate, dibutyl phthalate or a non-drying oil such as castor oil. On the other hand, binders which are not stiff enough can be modified by including inert fillers such as pulverized flint or they can be mixed with heat-hardening resins which are set up in the subsequent heat treatment of the abrasive coated articles. Selective variation of the flexibility may also be accomplished by selecting different resins having the desired properties. For example, a series of alkyd resins of varying flexibility may be used.

The method of producing composite material having a desired degree of flexibility is not limited to the use of thermoplastic resins but may include also the use of heat hardenable resins of varying flexibility. For example heat hardenable glycerol-dibasic acid alkyd resins may be used. A series of resins of varying flexibility may be prepared by mixing glyceryl phthalate and glycol succinate in varying ratios. In addition flexibilizing agents may be added to certain resins in varying proportions to produce resins of varying flexibility; for example, m-dinitrobenzene, and high boiling solvents such as diethyl

phthalate, triacetin, and aniline. Series of resins of uniformly varying flexibility may be used to produce a series of composite sheets of uniformly varying flexibility.

5 As indicated in the specific examples, one type of backing binder and a different type of abrasive grain binder may be used, or the two binders may be of the same general character. Likewise, it is possible to employ the same kind of binder in the 10 making or first coat of grain adhesive, and a binder of the same or of a different character as a second or sizing coat, which is applied after the abrasive grains have been attached to the backing by the making coat.

15 As indicated in the discussion of the prior art, my invention has a number of advantages. For example, it makes it possible to use cheaper materials in the backing than the vulcanized fiber which has been heretofore employed. It also 20 makes it possible to use binders for the abrasive grain which require heat treatment and which cannot be used in combination with backings united with glue. Furthermore it provides a 25 method of making backings having any desired degree of flexibility.

My improved backing also has the advantage that it can be readily flexibilized by merely heating. This is not true of backings which employ heat hardening resins as the backing binder 30 because such resins do not soften under heat and when the backing has once been combined and treated to set up the resin to a point where it is no longer sticky, it cannot be made sufficiently flexible so that it can be passed through the 35 usual abrasive paper-making machine.

As indicated, my invention is adaptable to a number of modifications and embodiments, and is not to be limited to the specific examples mentioned.

40 I claim:

1. The method of making a coated article which

is relatively stiff and rigid in its own plane but is capable of being repeatedly flexed by the application of lateral pressure which comprises adhesively uniting a plurality of webs of backing material by means of a cement which is relatively 5 stiff and inflexible at ordinary temperatures but capable of being made flexible and plastic by heating and of being alternately heated and cooled without causing a separation of the layers of backing material, thereby forming a composite 10 web which is so stiff at ordinary temperatures that it cannot be passed through an abrasive paper-coating machine but which can be flexibilized by heating to make it capable of being so passed, maintaining the composite web at a tem- 15 perature such that the web is flexible, passing the web through an abrasive paper-coating machine and coating it with abrasive and adhesive, and cooling the abrasive coated web.

2. The method of making a coated abrasive article which is relatively stiff and rigid in its own plane but is capable of being repeatedly flexed by the application of lateral pressure which comprises adhesively uniting a web of cloth and a web of a hydrated cellulose material by means 25 of a cement which is relatively stiff and inflexible at ordinary temperatures but capable of being made flexible and plastic by heating and of being alternately heated and cooled without causing a separation of the layers of backing mate- 30 rial, thereby forming a composite web which is so stiff at ordinary temperatures that it cannot be passed through an abrasive paper-coating ma- 35 chine but which can be flexibilized by heating to make it capable of being so passed, heating the composite web to a temperature such that the web is flexible, passing the web through an abra- 40 sive paper-coating machine and coating it with abrasive and adhesive, and cooling the abrasive coated web.

FRANK J. TONE.